

## UNITED STATES PATENT OFFICE

HENRY J. LORANG, OF ST. LOUIS, MISSOURI, ASSIGNOR OF ONE-HALF TO FRANK J. KUNA,  
OF ST. LOUIS, MISSOURI

## ZINC ALLOY

No Drawing.

Application filed July 18, 1929. Serial No. 379,330.

The general object of this invention is to provide a zinc alloy for use more particularly as bearing metal and which shall possess properties which render it markedly superior, 5 both from an economical and functional stand-point, to commercial bearing metals now on the market.

The characteristics which distinguish my improved alloy from other alloys used in 10 forming bearing metals are, low co-efficient of friction; small bearing temperature rise; great transverse strength; absence of material shrinkage in cooling; and satisfactory machining properties.

15 In producing the alloy, I first provide a fixed metal by mixing together equal parts by weight of copper and zinc. This, in reality, forms a brass. I then take one ounce of this fixed metal or brass and combine with 20 it fourteen ounces of zinc and one-half ounce of aluminum. The combined metals are, of course, melted together and the resultant product is a metal alloy about five times harder than zinc and having a melting point 25 but slightly greater than that of zinc. For purposes of comparison, it may be stated that the melting point of brass composed of equal parts by weight of copper and zinc is 1175° F.; that of aluminum is 1217° F.; and 30 that of zinc, 786° F. The melting point of my alloy is from 815° to 820° F.

Stated in terms of percentages by weight, my improved alloy is composed as follows:

Brass (equal parts of copper and zinc), 35 6-14/31%; Aluminum, 3-7/31%; Zinz (prime western), 90-10/31%.

The proportions of the metals named, I have found to give the most satisfactory results. However, the invention is not limited 40 to these exact proportions as, particularly in the case of zinc, the proportions named may be varied within reasonable limits without departing from the spirit of the invention and still produce a satisfactory bearing metal. 45 Referring particularly to the zinc ingredient, I may vary the quantity used relative to the other ingredients within a range extending from thirteen ounces to sixteen ounces; as stated, however, I prefer to use approximately 50 fourteen ounces.

Friction tests were conducted with bearing blocks machined from my improved alloy which were used in conjunction with a Riehle friction testing machine. The zinc alloy friction test was parallel with a similar 55 test using copper-tin-zinc bronze blocks, all test conditions being equal except the bearing blocks. Previous to the test run, my zinc alloy blocks were "run-in" under full lubrication for eight hours at full load. The test 60 run consisted of an eight-hour run beginning with the bearing at room temperature. Readings of the bearing friction and temperature rise were taken at frequent intervals 65 throughout the run. The readings showed the stabilized conditions of operation for the two alloys to be as follows:

|                                      | Zinc alloy | Bronze |
|--------------------------------------|------------|--------|
| Coefficient of friction.....         | .00221     | .00184 |
| Temperature rise of bearing—° F..... | 32.2       | 28.8   |

It will thus be seen that the friction characteristics of the zinc alloy used in this test approach those of a high-grade bearing 75 bronze.

The above test was conducted at the laboratories of the Massachusetts Institute of Technology, Cambridge, Massachusetts.

Tests for transverse strength were conducted at the testing laboratory of Washington University, St. Louis, Missouri, the comparison being between a zinc bar and a bar of my improved alloy. In this test, the zinc bar had a size of 1.1" x 1.0" and a bar of my 80 alloy had a size of 1.0" x 1-1/16". Both bars had a span of 3.5". The zinc bar sustained a central load of 1880 pounds, while the bar of my zinc alloy sustained a central 85 load of 9380 pounds, before breaking.

It will be observed that notwithstanding the superior qualities as a bearing metal possessed by my improved zinc alloy, I utilize a relatively low grade of zinc in its composition. Commercial deliveries of prime 90 western slab zinc analyze, as to constituents, about as follows:

Lead, .50-1.50; iron, .01-.08; cadmium, .10-.75.

The use of this grade of zinc thus enables 100

me to produce a very high-grade bearing metal at a relatively low cost, as compared with other bearing metals now on the market.

5 I claim:

1. The method of making a zinc alloy, which consists in forming a fixed metal by combining equal parts by weight of copper and zinc, and then combining with a given 10 quantity of said fixed metal aluminum and zinc, the resultant alloy having the metals combined in substantially the following percentages by weight, namely: fixed metal, 6-14/31%; aluminum, 3-7/31%; and zinc, 15 90-10/31%.
2. The method of making a zinc alloy which consists in forming a fixed metal by combining equal parts by weight of copper and zinc, and then combining said fixed metal 20 with aluminum and zinc in substantially the proportions of one ounce of the fixed metal to fourteen ounces of zinc and one-half ounce of aluminum.

In testimony whereof, I have hereunto set  
25 my hand.

HENRY J. LORANG.

30

35

40

45

50

55

60

65